

Aug. 16, 1938.

E. C. CHANCEY

2,126,734

HEATING PAD

Filed Aug. 31, 1936

Fig. 1.



Fig. 2.



Fig. 4.



Fig. 3.



Fig. 5.



INVENTOR:

Ernest C. Chancey  
by Caw & Caw & Chancey

HIS ATTORNEYS

## UNITED STATES PATENT OFFICE

2,126,734

## HEATING PAD

Ernest C. Chancey, Detroit, Mich.

Application August 31, 1936, Serial No. 98,717

3 Claims. (Cl. 132—36.2)

My invention relates to the type of pads that are used for applying heat to tresses of hair. The principal objects of the invention are to provide for the application of the heat at a temperature suitable for the hair and to maintain such temperature fairly uniform throughout the period of treatment. The invention consists principally in a composition of matter hereinafter described and claimed. It also consists in the combination of such composition with the package hereinafter described and claimed.

In the accompanying drawing wherein like reference numerals refer to like parts wherever they occur,

15 Fig. 1 is a view of a pad conforming to my invention;

Fig. 2 is a view of a sheet of bibulous paper used with said pad;

Fig. 3 is an enlarged fragmentary section 20 through said pad on the line 3—3 in Fig. 1;

Fig. 4 is a view showing the bibulous paper applied to the pad; and

Fig. 5 is an enlarged fragmentary section on the line 5—5 in Fig. 3.

25 My container comprises a rectangular sheet 1 of aluminum foil and a sheet 2 of unsized paper that is readily permeable by water. A suitable quantity of the composition 3 hereinafter described is placed between said sheets and the 30 margins thereof are folded together to close the container. A sheet 4 of bibulous paper is associated with each container.

The following formula represents a composition that is suitable for my invention, namely:

|                              | Grams |
|------------------------------|-------|
| Chlorate of potassium        | .90   |
| Aluminum dust                | 1.30  |
| Anhydrous sulphate of copper | .15   |
| Kaolin                       | 2.00  |
| Pumice                       | 2.00  |
| Total                        | 6.35  |

45 All of the ingredients are pulverized or finely divided and thoroughly mixed together. The total quantity represented by this formula is sufficient for a container of about two inches wide by three inches long.

In practical use, the sheet of bibulous paper 50 is dipped into water or otherwise wet with water and applied to the paper side of the package, which is then folded and clamped around the tress of hair. The water percolates through the paper side of the package, wets the composition 55 therein and brings about a reaction between the

chlorate of potassium and the metallic aluminum. Under ordinary conditions, this reaction would proceed slowly but, in my composition, this reaction is stimulated and quickened by the presence of copper sulphate, which acts as a catalyst but itself undergoes no chemical reaction.

The oxidation of the metallic aluminum generates considerable heat inside of the pad. Some of this heat converts some of the water into steam which acts to steam the tress of hair. Some of the heat is initially absorbed by the kaolin and pumice and later transmitted by them through the paper side of the package to the hair. The kaolin and the pumice are chemically inert; but they serve to prevent excessive rapidity of oxidation of the aluminum, they make it easy to distribute the small quantity of active chemicals throughout the package with a fair degree of uniformity, and they serve to first absorb considerable of the heat of reaction and later yield it to the hair over a limited period of time and at a substantially uniform temperature for the length of time required. It is noted that the aluminum foil, which constitutes the outer side or cover of the package, acts as an insulator and causes the greater portion of the heat of reaction to be transmitted through the inner side of the package.

In practice, I have found that the package hereinbefore described, containing 6.35 grams of 30 the composition conforming to the above mentioned formula, when wet with bibulous paper and bent around the hair in the usual manner, will produce a temperature of about two hundred eight degrees Fahrenheit, in the hollow 35 of the pad, within one minute and will maintain the heat there for about eight to ten minutes with only two or three degrees variation thereof during that time.

It is noted that, for several reasons, there is no 40 danger of burning the hair. First, while the temperature inside of the pad is high enough to convert water into steam, such conversion of water into steam absorbs considerable heat and the steam itself tends to protect the hair. Again, 45 water is required for the chemical reaction which generates the heat and when all the water is evaporated, chemical reaction ceases. Accordingly, the water-holding capacity of the bibulous paper is a factor in the ultimate results. In 50 practice, with the package above described, I have found it desirable to use bibulous paper with a water-holding capacity of about three cubic centimeters.

The particular composition hereinbefore de- 55

scribed is most suitable for use with medium fine hair. For treating finer hair, the temperature should be maintained for a longer period. For treating fine hair, I prefer the following composition:

|                       | Grams |
|-----------------------|-------|
| Chlorate of potassium | 1.30  |
| Aluminum dust         | 1.70  |
| Copper sulphate       | .15   |
| 10 Kaolin             | 1.50  |
| Pumice                | 3.50  |
|                       | <hr/> |
| Total                 | 8.15  |

15 This composition, in the quantity designated, and used with the needed water, will generate steam and will maintain an effective temperature on the tress therein somewhat above two hundred degrees Fahrenheit for a period of about twelve minutes.

20 For treating coarse hair, I prefer the following formula:

|                       | Grams |
|-----------------------|-------|
| Chlorate of potassium | .50   |
| Aluminum dust         | .80   |
| 25 Copper sulphate    | .15   |
| Pumice                | 3.00  |
| Kaolin                | 3.00  |
|                       | <hr/> |
| Total                 | 7.35  |

30 Coarse hair does not require as long steaming as finer hair and the formula last given will produce a temperature of about two hundred eight degrees Fahrenheit at the air in one minute after the wetting of the pad, which temperature drops in the course of five minutes to about two hundred degrees Fahrenheit.

For treating medium coarse hair, I prefer the following formula:

|                       | Grams |
|-----------------------|-------|
| Chlorate of potassium | .60   |
| Aluminum dust         | .80   |
| Copper sulphate       | .15   |
| Pumice                | 2.70  |
| 45 Kaolin             | 2.70  |
|                       | <hr/> |
| Total                 | 6.95  |

What I claim is:

1. A self-heating pad of the kind described comprising a single ply of aluminum foil and a single ply of absorbent paper with their margins folded to form a container, and a composition in said container substantially of the following formula:

|                              | Grams |
|------------------------------|-------|
| Chlorate of potassium        | .90   |
| Aluminum dust                | 1.30  |
| Anhydrous sulphate of copper | .15   |
| Kaolin                       | 2.00  |
| Pumice                       | 2.00  |
|                              | <hr/> |
| Total                        | 6.35  |

5

10

15

2. A self-heating pad of the kind described comprising a single ply of aluminum foil and a single ply of absorbent paper with their margins folded to form a container, and a composition in said container substantially of the following formula:

|                       | Grams |
|-----------------------|-------|
| Chlorate of potassium | 1.30  |
| Aluminum dust         | 1.70  |
| Copper sulphate       | .15   |
| Kaolin                | 1.50  |
| Pumice                | 3.50  |
|                       | <hr/> |
| Total                 | 8.15  |

20

25

30

35

3. A self-heating pad of the kind described comprising a single ply of aluminum foil and a single ply of absorbent paper with their margins folded to form a container, and a composition in said container substantially of the following formula:

|                       | Grams |
|-----------------------|-------|
| Chlorate of potassium | .50   |
| Aluminum dust         | .80   |
| Copper sulphate       | .15   |
| Pumice                | 3.00  |
| Kaolin                | 3.00  |
|                       | <hr/> |
| Total                 | 7.35  |

40

45

ERNEST C. CHANCEY.